

## UNITED STATES PATENT OFFICE

2,221,254

## MAGNESIUM BASE ALLOY

Joseph D. Hanawalt and John C. McDonald, Midland, Mich., assignors to The Dow Chemical Company, Midland, Mich., a corporation of Michigan

No Drawing. Application November 13, 1939,  
Serial No. 304,131

3 Claims. (Cl. 75—168)

This invention relates to magnesium base alloys. It more particularly concerns alloys of this nature having improved physical properties, such as high tensile and yield strengths associated with a sufficient degree of ductility or formability to permit relatively sharp bends to be made without the article developing external cracks.

Magnesium alloys are being widely used in various structural and mechanical arts, where a light weight metal is highly desirable, such as for use in making castings, forgings, and the like. However, the use of these alloys in the rolled form to make sheet metal articles requiring forming

high degree of ductility, do have exceptionally high tensile and yield properties, thus making them very suitable for use in casting operations. The following table, which lists some of the properties of sheet metal made from our new ternary alloy, as well as the properties of the related parent binary magnesium alloys having a similar composition, illustrates the improvement in strength characteristics of the new alloy over that of the related alloys. In the table the 10 per cent elongation is to be regarded as a measure of the ductility or formability of the alloys.

Table

| 20 | Nominal composition in percent (remainder—magnesium) |     | Annealed                       |                                  |                                | Cold rolled                    |                                  |                                | 20 |
|----|------------------------------------------------------|-----|--------------------------------|----------------------------------|--------------------------------|--------------------------------|----------------------------------|--------------------------------|----|
|    | Mn                                                   | Sr  | Yield strength in lbs./sq. in. | Tensile strength in lbs./sq. in. | Percent elongation in 2 inches | Yield strength in lbs./sq. in. | Tensile strength in lbs./sq. in. | Percent elongation in 2 inches |    |
| 25 | 2                                                    | 0.6 | 19,000                         | 33,000                           | 4                              | 23,000                         | 31,000                           | 2                              | 25 |
|    | 3                                                    | 0.5 | 16,000                         | 30,000                           | 9                              | 24,000                         | 31,000                           | 3                              |    |
|    |                                                      |     | 23,000                         | 35,000                           | 9                              | 27,000                         | 34,000                           | 5                              |    |

operations, such as bending, drawing, and the like, has not progressed as rapidly, due to the fact that, in general, alloys of good formability do not possess the most desirable characteristics 30 as regards their yield and tensile strengths.

It is accordingly the principal object of the invention to provide a magnesium base alloy which may be rolled into sheet or the like, possessing a sufficient degree of ductility or formability to be bent, drawn, or otherwise shaped and still possess high tensile and yield strengths.

Other objects and advantages of the invention will be apparent as the description of the invention proceeds.

40 Our invention resides in the discovery that a magnesium base alloy composed of from 0.1 to 3 per cent of manganese and from 0.05 to 1 per cent of strontium, the balance being substantially all magnesium, is endowed with the afore-mentioned properties. While the properties of high tensile and yield strengths, together with a sufficient degree of formability, are manifest over the entire range of composition indicated, we have found that, in general, the preferred combination of properties, such as high tensile and yield strengths coupled with good ductility, is found in alloys containing from 1 to 3 per cent of manganese and from 0.1 to 0.6 per cent of strontium. Alloys containing the higher percentages of alloying ingredients, while not possessing such a

25 The properties listed in the above table under the section headed by the term annealed were obtained by first rolling the alloys at a temperature between about 600° to 800° F., and thereafter annealing them at various temperatures 30 through a temperature range of from 400° to 800° F. The properties selected for the table were those of the annealed specimens which exhibited the maximum elongation. The properties listed under the section headed cold rolled were obtained by subjecting specimens of the alloys which had been hot rolled at a temperature of from 600° to 800° F. to additional rolling in the cold state, to bring about a total reduction in thickness of from 2 to 10 per cent. The properties selected for the table were those of the cold rolled specimens which showed the greatest tensile and yield strengths, while having at least a 1 per cent elongation in 2 inches.

40 By a comparison of the properties listed in the above table, it will be observed that the combined properties of our new ternary alloy are superior to those of the present binary magnesium alloys having comparable percentages of alloying ingredients. For example, it will be noted that in the annealed state the specimen showed a marked improvement in yield strength over that of the related binary alloys without any loss in per cent elongation. Similarly the

5 tensile strength showed a marked improvement. This improvement is also apparent in the cold rolled state where the new ternary alloy shows improvement in yield and tensile properties, as well as in elongation. Similarly in other portions of the composition range improvement in these properties will also be observed. Further, the new alloy has highly desirable characteristics as regards resistance to corrosive conditions.

10 10 While the alloy is most useful in wrought form, such as sheets due to its formability characteristics it may also be suitably used in making castings, forgings, extruded forms and the like.

15 15 The new alloy may be compounded in any of the ways known to the art, such as by adding the alloying ingredients to the molten magnesium under a suitable flux. The flux should be free from magnesium chloride if the strontium content of the alloy is to be above about 0.4 per cent.

20 20 In those instances where an alloy is to be com-

pounded containing less than 0.4 per cent of strontium, magnesium chloride may be present in the flux, without exerting deleterious effect, but in this case it is usually preferable to add the strontium last and without too much stirring 5 in order that the loss of strontium into the flux will be substantially prevented.

We claim:

1. A magnesium base alloy containing from 0.1 to 3 percent of manganese and from 0.05 to 1 10 per cent of strontium, the balance being magnesium.

2. A magnesium base alloy containing from 1 to 3 per cent of manganese and from 0.1 to 0.6 per cent of strontium, the balance being magnesium. 15

3. A magnesium base alloy containing from 1 to 2 per cent of manganese and 0.5 per cent of strontium, the balance being magnesium.

JOSEPH D. HANAWALT.

JOHN C. McDONALD. 20